

Jan. 31, 1950

W. W. URMETZ

2,495,992

INGOT MOLD AND HOT TOP

Filed June 28, 1946



FIG. 1

FIG. 2



FIG. 4



INVENTOR.

WALTER W. URMETZ  
BY

Kivis, Hudson, Boughton & Williams  
ATTORNEYS

## UNITED STATES PATENT OFFICE

2,495,992

## INGOT MOLD AND HOT TOP

Walter W. Urmetz, Parma, Ohio, assignor to The  
Ferro Engineering Company, Cleveland, Ohio,  
a corporation of Ohio

Application June 28, 1946, Serial No. 680,260

6 Claims. (Cl. 22—139)

1

This invention relates to improvements in killed steel ingots and to a method and apparatus for casting the same.

Killed steel ingots are cast in molds provided with hot tops in order that a pool of molten metal may be maintained to flow downward and fill the cavity or piping which tends to form in the upper end of the ingot, centrally thereof, as contraction or shrinkage occur due to cooling. Solidification of some of the metal originally held in the hot top takes place unavoidably, and then constitutes what is known in the art as a sinkhead. Since the sinkhead is waste metal and must be cropped off, it is obviously desirable to limit its mass as much as conditions will permit. However a certain minimum height of hot top is necessary in order to maintain a proper head of metal to insure rapid flow, and a certain minimum content of hot topped metal is necessary to make sure that the molten metal in the hot top will not be entirely expended before freezing of the ingot body is completed.

This minimum hot top capacity varies somewhat with the grade of steel, but the important factor is the degree of insulation provided by the hot top. With a hot top body or lining of high insulating quality the size of the hot top may be reduced with a consequent important saving of metal.

In accordance with the present invention the mold is formed big end down, and is necked-in at its upper end and provided with a central opening which may be of considerably less area than the cross-sectional area of the ingot. A hot top is disposed in operative relation with this opening. The shoulders formed in the ingot body by this necking-in may be given contours such as to minimize fishtailing, following approved practice for the bottom ends of ingots.

The present invention has special advantages in connection with slab molds, for the necking-in of such molds may be principally or entirely from the narrow sides of the mold, so that the two dimensions of the mold opening may be made equal if desired and the hot top may then be square or round, which of course is ideal from the standpoint of a minimum surface of radiation in proportion to the volume of metal hot topped.

Bottleneck molds, so called, are used extensively in the making of rimmed steel, without hot tops, but there they have very special functions, that is to say the constricted opening is convenient in that it limits the size of the cap for sealing the opening, and also the rounded

2

shoulders of the mold form strong walls against which the heavy pressure exerted by the "growing" metal expends itself, thereby pressing the gas in the metal away from the skin of the ingot and toward the axis thereof.

The necking-in of the mold in accordance with my invention is for an entirely different purpose, and the shouldered portions need not be thick and strong since in killed steel ingots there is no heavy pressure to be resisted. In the case of my invention the necked-in portions are for the purpose of accommodating a relatively small and efficiently designed hot top, and in order to provide an end contour for the ingot which will maintain at a minimum the cropping necessary after rolling.

An object of the invention therefore is the provision of a new method and means for casting ingots of killed steel more efficiently, to give a greater yield of usable metal.

Another object is the provision of a novel and useful combination of hot top and necked-in mold, for the purpose stated.

A further object is the production of a killed steel ingot of a form which may be rolled efficiently.

Other objects and features of novelty will appear as I proceed with the description of that embodiment of the invention which, for the purposes of the present application, I have illustrated in the accompanying drawing, in which

Fig. 1 is a vertical sectional view through a slab mold and hot top embodying the invention, the view being taken through a central plane between the wide sides of the mold, as indicated by the line 1—1 of Fig. 3.

Fig. 2 is a vertical sectional view at right angles to that of Fig. 1, as indicated by the line 2—2 of Fig. 3.

Fig. 3 is a plan view of the mold and hot top, and

Fig. 4 is a fragmental vertical sectional view taken diagonally of the mold and hot top substantially on the line 4—4 of Fig. 3.

In the drawing, 10 represents a mold stool upon which is supported a big end down mold 11. In the illustrated case the mold is a slab mold having two wide sides 12 and two narrow sides 13. All four sides taper somewhat toward the top of the mold in order to provide the necessary draft.

The upper end of the mold is constricted by two shoulders or necked-in portions 14 which extend inwardly from the upper ends of the narrow side walls 13. These necked-in portions

may be relatively thin as compared with the walls 12 and 13. Curved surfaces 15 of relatively long radii join the inner surfaces of these shoulders with the inner surfaces of the narrow side walls of the mold. These shoulders extend inwardly far enough to form a constricted opening 16 with a dimension parallel to the wide sides of the mold which may be substantially the same as the distance between the narrow sides. In such case the opening 16 is substantially square. It may be of a shape other than square, but it should be symmetrical and its horizontal dimensions parallel to the sides of the mold are preferably equal. The area of the mold just below the shoulders is indicated by broken lines at 17 in Fig. 3. In the event that a floating hot top is to be used the mold should have a neck 9.

When an ingot is to be poured I mount a hot top upon the mold in operative relation with the opening 16. Any conventional hot top may be employed. For purposes of illustration I have shown herein a composite hot top of the full floating type extending down into the opening 16. 20 represents a metal casing the lower portions of which are of a size and shape to fit the opening 16 with clearance between the casing and the mold, which clearance may be taken up by flexible sheet metal wiper strips, not shown, which are well-known in the art. The metal casing 20 is provided with an upper semi-permanent refractory lining 21 having heat insulating qualities, and the lower end of the casing is protected by a refractory bottom ring 22.

The ingot body is marked 25 in the drawing and the sinkhead 26 is shown with its shrinkage cavity 27.

The shrinkage cavity tending to form in the ingot body during solidification is concentrated near the vertical center line of the ingot. Hot topping the central part of the mold only therefore fulfills the requirement insofar as supplying feed metal is concerned. The fact that the hot top as herein illustrated has substantially equal horizontal dimensions at right angles to each other is advantageous in that for a given volume of hot topped metal the wall surface and top area exposed to cooling is of minimum extent. Consequently there is minimum loss from solidification of metal in the hot top.

The constriction at the top of the mold provides the means of forming an ingot with an upper end contour similar to that contour of the butt end of a big end up mold, which has been found in practice to be advantageous for rolling in respect to minimizing the amount of loss from cropping.

Although the invention is herein illustrated as applied to a slab mold, it should be understood that in its broader aspects it is equally applicable to molds of any cross-sectional proportions, and that the necking-in of the mold may be effected from all four sides rather than from two sides as herein shown.

Having thus described my invention, I claim:

1. In combination, a big end down slab ingot mold having wide sides and narrow sides, the upper end of said mold being necked-in from said narrow sides and having a central opening of approximately equal dimensions parallel to said wide and narrow sides, and a hot top of approximately equal horizontal dimensions disposed in operative relation with said opening and extending upwardly therefrom.

2. In combination, a big end down slab ingot mold having wide sides and narrow sides, the

upper end of said mold being necked-in from said narrow sides and having a central substantially square opening, and a substantially square hot top disposed in operative relation with said opening and extending upwardly therefrom,

3. In combination, a big end down slab ingot mold having wide sides and narrow sides, the upper end of said mold being necked-in from said narrow sides and having a central opening of cross-sectional dimensions approximately the same as the internal width of the mold adjacent the opening, and a hot top of approximately equal horizontal dimensions disposed in operative relation with said opening and extending upwardly therefrom.

4. In combination, a big end down slab ingot mold having wide sides and narrow sides, the upper end of said mold being necked-in from said narrow sides and having a substantially square central opening of cross-sectional dimensions approximately the same as the internal width of the mold adjacent the opening, and a substantially square hot top disposed in operative relation with said opening and extending upwardly therefrom.

5. In combination, a big end down slab ingot mold having wide sides and narrow sides, the upper end of said mold having shoulders extending inwardly from said narrow sides, the internal surfaces of said shoulders being well rounded, the upper end of the mold having an opening between said shoulders of approximately equal dimensions parallel to said wide and narrow sides, and a hot top of approximately equal horizontal dimensions disposed in operative relation with said opening and extending upwardly therefrom.

6. In combination, a big end down slab ingot mold having wide sides and narrow sides, the upper end of said mold having shoulders extending inwardly from said narrow sides, the internal surfaces of said shoulders being well rounded, the upper end of the mold having an opening between said shoulders of approximately equal dimensions parallel to said wide and narrow sides, and a hot top of the full floating type of approximately equal horizontal dimensions extending into said opening.

WALTER W. URMETZ.

#### REFERENCES CITED

The following references are of record in the file of this patent:

#### UNITED STATES PATENTS

| Number    | Name      | Date          |
|-----------|-----------|---------------|
| 385,836   | Boucher   | July 10, 1888 |
| 644,740   | Griffith  | Mar. 6, 1900  |
| 1,055,833 | Talbot    | Mar. 11, 1913 |
| 1,417,246 | Hazeltine | May 23, 1922  |
| 1,603,662 | Coates    | Oct. 19, 1926 |
| 1,720,857 | Perry     | July 16, 1929 |
| 1,804,206 | Charman   | May 5, 1931   |
| 2,190,392 | Belding   | Feb. 13, 1940 |

#### OTHER REFERENCES

"The Making, Shaping and Treating of Steel," page 652, pub. by Carnegie-Illinois Steel Corp., Pittsburgh, copyright 1940.

Gathmarn: "The Ingot Phase of Steel Production," pages 18 and 19. Copyrighted in 1942. Printed by Schneidereith & Sons, Baltimore, Md.